

## UNITED STATES PATENT OFFICE.

ARTHUR S. O'NEIL, OF EAST ALTON, ILLINOIS, ASSIGNOR TO WESTERN CARTRIDGE COMPANY, OF EAST ALTON, ILLINOIS, A CORPORATION OF DELAWARE.

## PROPELLANT POWDER AND PROCESS FOR MAKING SAME.

No Drawing.

Application filed February 10, 1923. Serial No. 618,3882

This invention relates to propellant powders, and more particularly to nitro-cellulose powders adapted for use in and suitable for cylinder guns and small arms.

5 Smokeless powder having a nitrocellulose base, adapted for rifle fire arms and more particularly for use as military ammunition, is made generally in the following manner: Cotton or cellulose, after preliminary washing, etc. is nitrated with a mixture of nitric and sulfuric acid and then washed with water. The nitrocellulose so produced can be either a soluble or a mixture of soluble and insoluble nitrocellulose (that is, soluble wholly or partially in ether-alcohol), depending upon the degree of nitration.

10 The nitrocellulose is then dehydrated by displacing the water with alcohol in a dehydrating press. The dehydrated product has then added thereto ethyl-ether together with a stabilizer, such as diphenylamin, and the whole mixed or incorporated so as to form a colloid. This colloid is then formed into blocks, pressed through dies to form 15 strings and the strings can be cut to form the grains. The grains are then placed in a solvent recovering apparatus to recover the solvent and are then dried.

20 The above process forms a dense nitrocellulose colloid which burns progressively, that is, in layers until completely consumed. While it is, therefore, peculiarly adapted for rifle arms where the projectile seals the bore, it is not suitable for cylinder guns and 25 small arms. In powders for cylinder guns, it is necessary that the initial burning be at a more rapid rate, due to the fact that the bore of the gun is not sealed by the projectile. Accordingly if the pressure is not rapidly developed, incomplete burning results, since the rapidity of burning depends directly upon pressure. Accordingly, where 30 a dense nitrocellulose powder is employed in a cylinder gun, the result will be unburnt powder and escape of the gases around the wads, thereby reducing the ballistic efficiency.

In the preparation of nitrocellulose powder for use as military ammunition, it has

further been the practice to subject the dense 50 nitrocellulose colloid to surface treatment by coating or impregnating the same with a suitable nitro-hydrocarbon, thereby producing a so-called progressive powder having a still lower initial pressure without, 55 however, lowering the velocity of the projectile. The function of the solvent, however, is to act as a deterrent, as this solvent is not only less explosive and less readily ignitable than the dense nitrocellulose colloid, but it acts as a seal; it will, therefore, be seen that this surface treatment goes still further in the opposite direction than the requirements and characteristics desired in a powder suitable for use in cylinder guns 65 and small arms.

In order to produce a smokeless powder having a nitrocellulose base, it has been the practice heretofore to either mix with the nitrocellulose, metallic nitrates or a more 70 violent explosive ingredient, such as nitroglycerin. The former, however, produces smoke, while both have a corrosive action on the bore of the gun. It has also been the practice to employ weak solvents so as 75 to only partially gelatinize the nitrocellulose, or to employ ingredients with the nitrocellulose while in a plastic state which are subsequently extracted. These, however, are 80 open to the objection that they do not provide stable and uniformly burning grains. It has also been proposed to incorporate with smokeless powder, either by mixing therewith or as a supplementary priming charge, black powder or to cause the black powder 85 to adhere to the nitrocellulose powder grains by a binder. These, however, are not only open to the objection that they introduce smoke forming and corrosive constituents, but the black powder is liable to segregate 90 during shipment, thereby causing a given charge to be ununiform.

One of the objects of this invention, therefore, is to provide a propellant powder and more particularly one having a dense nitrocellulose colloid as a base, together with a process of making the same, whereby the surface of the powder grain is so modified

that it will approach the rate of burning of the so-called bulk powders, and in order that this rate of burning may be so accelerated that the initial pressure is developed at the rate required to enable its utilization and render it suitable for cylinder guns and small arms.

There are at the present time large quantities of military ammunition, both surface treated and untreated, which have no present use. It is not economical to keep such powder in storage, especially since it deteriorates and it is entirely unsuitable for peace and economic purposes.

Another object of this invention, therefore, is to provide a process adapted for the treatment of military smokeless powders so as to permit their utilization in and render them suitable for cylinder guns and small arms, and to so modify such military powder that the rate of burning is accelerated in order that the pressure may be developed more readily. The process is not, however, restricted to the treatment of dense military powders which have been salvaged, but it is adapted to the treatment of freshly prepared dense nitrocellulose powders.

Further objects will appear from the detail description in which are given a number of examples illustrating embodiments of this invention.

In accordance with this invention the powder grain is modified so as to form a dense core surrounded by a less dense and porous envelope. This is accomplished by swelling the surface of the grain to the desired depth of penetration and the swollen envelope so formed is then fixed. This fixing is accomplished in such a manner as to cause not only interruption of the swelling in order to secure an envelope of the desired depth, but also to break up the surface in order to leave an open and porous envelope which is readily ignitable.

Generally stated the dense nitrocellulose colloid is subjected to the action of a solvent which, upon penetration into the grain, causes an envelope to be formed which is less dense than the body of the dense colloid, and the solvent action is continued until the desired depth of penetration and the desired envelope thickness has been obtained. The action is then interrupted in such a manner as to not only limit the penetration, but so as to also produce an envelope which is not only less dense than the core which it surrounds, but such envelope is also porous and broken up so as to be readily ignitable, and the envelope is fixed in that condition.

In order to further explain the practical application and utility of this invention, an example of a practical embodiment of the process will be described, and we will assume as a base material a dense colloided nitrocellulose powder, such as standard untreated

military ammunition, although the process is equally applicable to freshly prepared nitrocellulose powders.

The powder is ground or cut up in any suitable apparatus to the state of division desired and it is then screened to the desired size. This powder is then intimately mixed with a solid nitro-hydrocarbon, such as dinitro-toluene, in the proportion of ninety-eight (98) parts of the powder and two (2) parts of the solvent, although the proportions may be varied within limits to suit requirements. The mixture is then introduced into a tank provided with a stirring mechanism, or into a tumbling barrel, which tank or barrel has been previously filled with water and raised to a temperature of 75° to 100° C., depending upon the nature of the solvent used. The temperature is maintained (by supplying live steam or water to a jacket or by the direct action of steam) for a suitable period, in case where dinitrotoluene is used for a period of about two hours, while the powder and the solid solvent are rumbled together in the water. The solvent under the influence of heat melts and distributes itself uniformly over the grain. Now dinitro-toluene (as well as other solid nitro-hydrocarbon solvents) under the influence of heat is a solvent and a colloiding agent for nitrocellulose. Accordingly the solvent penetrates the powder grain, the depth of penetration depending upon the period of heating, the quantity of the solvent, and the temperature of the heat applying vehicle. It is essential that the penetration takes place rather rapidly, otherwise little or no swelling of the grain takes place. It is also essential that the temperature be maintained until the desired penetration takes place.

The resulting grain then comprises a core of dense powder enclosed by an envelope of nitrocellulose colloided with dinitro-toluene, which in common with such colloids occupies a greater volume and is less dense than the core or body of the grain. It is, however, necessary to fix this condition and in order to accomplish this, the solvent action is not only interrupted but the powder grain is chilled. When, therefore, the colloiding and swelling action has progressed as far as desired, cold water is admitted to the mixture in order to rather suddenly chill the contents of the tank or barrel. This causes the dinitro-toluene to chill, thereby partially recrystallizing and losing its solvent properties so that the solvent action is interrupted. At the same time, a portion of the nitrocellulose is partially precipitated from the colloid, while the dinitro-toluene is also partially precipitated. Accordingly the envelope, which before the chilling consisted of nitrocellulose colloided with dinitro-toluene, will become partially decolloided. The chilling

of the envelope not only causes it to crack and become porous, but the precipitation of the nitrocellulose and the dinitro-toluene from the colloid of the envelope enhances 5 the porosity and broken formation of the surface. The result is, therefore, that there is produced a powder grain which not only has a greater volume than the original dense nitrocellulose colloid, but it retains the 10 dense colloid core while the envelope is less dense than the core and porous. The porous formation of the surface not only causes the powder grain to ignite more readily but the particles of precipitated nitrocellulose are 15 more readily ignitable than was the original dense colloid. The structure of the envelope is, therefore, such that it is not only readily ignitable, but it will continue to burn at a higher rate under a reduced pressure, so that 20 the burning of the envelope supplies the necessary temperature and pressure to afford complete combustion of the balance of the grain. This rate of combustion can be regulated by variation of the thickness of the 25 envelope, which can readily be controlled by extending the penetration period of the solvent.

It will, of course, be understood that after chilling the treated grains are removed from 30 the water and dried in the usual manner. This drying will not, however, cause contraction of the envelope to the original colloid density, but this envelope will remain in a porous condition since the drying will 35 rather enhance than detract from the porosity. The drying can be accomplished in any suitable manner as usual in the art.

If a coated powder is desired, additional 40 dinitro-toluene may be added after chilling, the water reheated until the solvent is melted and distributed over the surface and chilling again proceeded with.

While in the above described embodiment 45 of the process dinitro-toluene has been described as a solvent, it is understood that other solid solvents may be used, such as dinitro-benzene, nitro-naphthalene or other solid nitro-hydrocarbons. The procedure when using such solvents is similar to that 50 described above.

It is also possible to obtain improved results by employing diluted volatile solvents, such as acetone, ketones, wood alcohol, etc. When using volatile solvents, however, the 55 dense powder is subjected to the action of the volatile solvents, either in water or in the presence of another liquid which is indifferent to nitro-cellulose. The action of this solvent causes the grains to swell and increase in volume, and the treatment is continued until the desired penetration has been effected. The treated grains are then quickly immersed in hot water which causes violent expulsion of the solvent; the grains so 60 treated may then be chilled by dropping

them in cold water. The grains may then be dried in any suitable manner.

It will thus be seen that the invention accomplishes its objects. A powder is obtained which comprises a core of a dense nitrocellulose colloid which is enveloped by a less dense and porous envelope, which envelope being further decolloided, and parts of the broken and porous surface containing uncolloided nitrocellulose which is readily ignitable, and an uncolloided combustible solvent. The result, therefore, is a powder grain whose surface is readily ignitable, so that its combustion is not only started at low pressure, but the envelope supplies and 70 maintains the necessary heat and pressure to secure and maintain the requirements for complete combustion of the dense core. Moreover the character and formation of the surface and envelope remains fixed even 75 after drying. Moreover the volume of the powder grains is considerably higher than that of the original dense colloided nitrocellulose, which is desirable. Thus, a standard three (3) dram measure of the powder embodying this invention is found to weigh 80 46.1 grains, while a three (3) dram measure of dense nitrocellulose powder weighs 54.2 grains. It will further be noted that the desired result is obtained without the mixture 85 of smoke forming or corroding ingredients, since the resultant grain is itself modified by modifying the density, porosity and character of the surface of the nitrocellulose colloid.

While in the specification and claims the term "grain" is used, it is to be understood that it is intended as a word of general description and not of limitation, but to include the various forms in which powder is 90 produced for use. It will be further understood that while theories of formation and operation have been advanced, the invention is not necessarily limited thereto. It will further be obvious that various changes may 95 be made in details without departing from the spirit of this invention; it is, therefore, to be understood that this invention is not to be limited to the specific details described.

Having thus described the invention, what 100 is claimed is:

1. A propellant powder grain comprising, a dense core surrounded by a porous envelope.
2. A propellant powder grain comprising, 105 a dense colloid, the surface of which is porous.
3. A propellant powder grain comprising, a dense colloid, the surface of which is partially decolloided.
4. A propellant powder grain comprising, 110 a dense colloid, the surface of which is colloided with a solvent so as to provide an envelope which is less dense than the core.
5. A propellant powder grain comprising, 115

- a dense colloid, the surface of which is colloided with a solvent so as to provide a porous envelope.
6. A propellant powder grain comprising, a dense colloid, the surface of which is partially decolloided and contains a combustible solvent.
7. A powder grain comprising, a dense nitrocellulose core surrounded by a porous envelope.
8. A powder grain comprising, a dense nitrocellulose core surrounded by a porous envelope containing a solvent.
9. A powder grain of dense colloided nitrocellulose, the surface of which is less dense than the core.
10. A powder grain of dense colloided nitrocellulose, the surface of which is partially decolloided so as to be readily ignitable.
11. A powder grain of dense colloided nitrocellulose, the surface of which is colloided with a solvent and is less dense than the core.
12. A powder grain of dense colloided nitrocellulose, the surface of which is porous so as to be readily ignitable.
13. A powder grain of dense colloided nitrocellulose, the surface of which is colloided with a solvent and chilled.
14. A powder grain of dense colloided nitrocellulose having a chilled colloided surface.
15. A powder grain of dense colloided nitrocellulose, the surface of which contains a precipitated nitro-hydrocarbon.
16. A powder grain of dense colloided nitrocellulose, the surface of which contains precipitated nitrocellulose.
17. A powder grain of dense colloided nitrocellulose, the surface of which contains precipitated nitrocellulose and a nitro-hydrocarbon solvent.
18. In the art of making propellant powder, the process comprising, swelling the surface of the grain and fixing the envelope so formed.
19. In the art of making propellant powder, the process comprising, swelling the surface of the grain and chilling the envelope so formed.
20. In the art of making propellant powder, the process comprising, subjecting the grain to the action of a solvent for the grain material and precipitating the solvent.
21. In the art of making propellant powder, the process comprising, subjecting the surface of the grain to the action of a solvent for the grain material and expelling the solvent.
22. In the art of making propellant powder, the process comprising, heating a grain, the surface of which contains a solvent and chilling the grain.
23. In the art of making propellant powder, the process comprising, swelling the surface of a dense nitrocellulose colloid and fixing the envelope so formed.
24. In the art of making propellant powder, the process comprising, swelling the surface of a dense nitrocellulose colloid and chilling the envelope so formed. 70
25. In the art of making propellant powder, the process comprising, partially decolloiding the surface of a dense nitrocellulose colloid. 75
26. In the art of making propellant powder, the process comprising, subjecting a dense nitrocellulose colloid to the action of a swelling medium and interrupting the swelling so as to fix the envelope so formed. 80
27. In the art of making propellant powder, the process comprising, subjecting a dense nitrocellulose colloid to the action of a solvent and interrupting the solvent action so as to fix the envelope so formed. 85
28. In the art of making propellant powder, the process comprising, subjecting a dense nitrocellulose colloid to the action of a swelling medium and expelling the medium from the envelope so formed. 90
29. In the art of making propellant powder, the process comprising, treating a dense nitrocellulose colloid with a solvent for nitrocellulose and precipitating the solvent. 95
30. In the art of making propellant powder, the process comprising, colloiding the surface of a dense nitrocellulose colloid with a solvent for nitro-cellulose and fixing the envelope so formed. 100
31. In the art of making propellant powder, the process comprising, colloiding the surface of a dense nitrocellulose colloid with a solvent and partially decolloiding the envelope so formed. 105
32. In the art of making propellant powder, the process comprising, heating a dense nitrocellulose colloid in the presence of a solvent and chilling the envelope so formed.
33. In the art of making propellant powder, the process comprising, heating a dense nitrocellulose colloid in the presence of a nitro-hydrocarbon solvent and chilling the envelope so formed. 110
34. In the art of making propellant powder, the process comprising, heating a dense nitrocellulose colloid in the presence of a solvent and a vehicle and chilling the envelope so formed. 115
35. In the art of making propellant powder, the process comprising, heating a dense nitrocellulose colloid in the presence of a nitro-hydrocarbon in water and chilling the envelope so formed. 120
36. In the art of making propellant powder, the process comprising, treating a dense nitrocellulose colloid with a nitro-hydrocarbon first in hot water and then in cold water. 125
37. In the art of making propellant powder, the process comprising, treating a dense nitrocellulose colloid with a solid nitro- 130

hydrocarbon first in hot water and then in cold water.

38. In the art of making propellant powder, the process comprising, rumbling a dense nitrocellulose colloid with a solid solvent in hot water and then treating the resulting 10 colloid with cold water.

39. In the art of making propellant pow-

der, the process comprising, rumbling a dense nitrocellulose colloid with a solid solvent in hot water and then treating the resulting 10 colloid with cold water.

In testimony whereof I affix my signature this 31st day of January, 1923.

ARTHUR S. O'NEIL.